

# UNITED STATES PATENT OFFICE.

JOSEF MÜLLER, OF SCHÖNAU, NEAR SCHLUCKENAU, AUSTRIA-HUNGARY.

## TREATING SHEET METAL BY ELECTROLYSIS.

No. 862,409.

Specification of Letters Patent.

Patented Aug. 6, 1907.

Application filed April 18, 1906. Serial No. 312,493.

*To all whom it may concern:*

Be it known that I, JOSEF MÜLLER, a subject of the Emperor of Austria, residing at Schönau, near Schluckenau, in the Kingdom of Bohemia and Empire of Austria-Hungary, have invented a new and useful Process 5 of Treating Sheet Metal and Depositing Metallic Coatings Thereon by Electrolysis, of which the following is a specification.

My invention relates to a process of treating sheets or 10 plates of metal and providing the same with metallic coatings by electrolysis.

For coating sheets or plates by electrolysis they have heretofore been ground, cleaned, suspended in the baths and polished separately. This separate treatment 15 of the sheets or plates is not only troublesome and, owing to the interruptions continually required, takes much time, but does not, even if carried out with the greatest care, give uniform coatings either on the same plate or on the several plates. This is partly due 20 to the fact that the plates are again and again brought in contact with the atmospheric air between each two steps of the treatment, and that they become otherwise soiled by being touched during transport or during the several steps of the treatment. For the most 25 part the defective uniformity of the coatings is however due to the plates being suspended singly in the electrolytic bath. The cause of this is that the plates are suspended by tongs or grippers which serve at the same time for admitting the current, the current being thus 30 admitted only at single points and not therefore distributed uniformly over the whole plate. Moreover, the plates can never be placed to their whole extent exactly parallel to the anodes by means of the tongs or grippers, and even if this were possible approximately, 35 they become bent by the action of the electric current, so that an exactly equal distance throughout between them and the anode, such as is requisite for the uniformity of the coating, is not obtainable. By my said invention I obtain the continuous working without any 40 interruption, the several operations follow each other immediately, and perfectly uniform coatings are deposited upon each single plate as well as upon the several plates, these plates being firmly connected with each other by welding, soldering, riveting, bolting, 45 clamping or otherwise securing their overlapping ends together, to form one continuous band of sheet metal which can be preliminarily treated, provided with the metallic coating and subsequently treated in the same manner as is already known for narrow metal 50 strips and bands.

The plates pass through the several devices and baths in proper order without interruption and almost without coming in contact with the atmospheric air. They are not at all liable to become soiled by being touched during the treatment. The plates connected 55 together to form a band pass over guide rollers and have a sufficient tension imparted to them by the pull whereby they are carried along, to preclude the bending of the plates by the action of the electric current. The guide rollers and thus also the plates may be 60 easily placed exactly parallel to the anodes. Furthermore, the guide rollers serve, in the manner already known, for the admission of the current, so that such admission will take place uniformly over the whole sectional area of the plate. Accordingly I produce 65 upon the plates a perfectly uniform coating which is not subjected to any detrimental action.

By the treatment of the sheets or plates in the form of a continuous band, as compared with the single treatment, a great saving in manual labor is insured, 70 and the production of plates having metallic coatings is considerably cheapened. The labor necessary for transporting the several plates from one device to another is entirely dispensed with, and several workmen can moreover be dispensed with who were heretofore 75 needed for attending to the several devices.

A special advantage consists in completely obviating interruptions of the current, together with the deleterious effects which they have upon the baths, which interruptions have hitherto been necessary when exchanging the several plates.

When the plates are finished they may be separated from each other by the removal of the connections. The finished plates do not show any rough places where the tongs or grippers were applied, so that in the preparation of the plates at most one centimeter of each of the overlapping plates will be wasted instead of three or five centimeters through the employment of tongs or grippers.

What I claim as my invention, and desire to secure 90 by Letters Patent, is—

The herein described process of electro-plating a plurality of individual sheets or plates, which consist in temporarily connecting the edges of said plates to form a continuous band and then passing the band continuously 95 through the electrolyte, substantially as described.

In testimony whereof I have signed my name to this specification in the presence of two subscribing witnesses.

JOSEF MÜLLER.

Witnesses:  
W. RÖNDT.  
ALFR. FOHLMAYER.